

Aug. 30, 1932.

A. MEISSNER

1,875,087

PIEZO ELECTRIC OSCILLATOR

Filed July 7, 1928

*Fig. 1*



*Fig. 2*



*Fig. 3*



INVENTOR  
ALEXANDER MEISSNER  
BY *Dr. J. Adams*  
ATTORNEY

## UNITED STATES PATENT OFFICE

ALEXANDER MEISSNER, OF BERLIN, GERMANY, ASSIGNOR TO TELEFUNKEN GESELLSCHAFT FÜR DRAHTLOSE TELEGRAPHIE M. B. H. HALLESCHES, OF BERLIN, GERMANY, A CORPORATION OF GERMANY

## PIEZO ELECTRIC OSCILLATOR

Application filed July 7, 1928, Serial No. 291,089, and in Germany July 19, 1927.

This invention relates to the piezo electric art and deals more specifically with a method of cutting quartz crystal oscillators from the native crystal.

Through investigations of the oscillations of a piezo electric crystal, I have discovered that there exists in a natural quartz crystal structural planes both at an angle of 40°-50° and 60°-75° approximately with respect to the optical axis, and these structural planes extend substantially through the whole structure of the crystal. These structural planes are preferential planes and are characterized by the fact that in the plane approximately 10 70° with respect to the optical axis the speed of propagation of sound is of the order of magnitude of 5400 meters per second and in the structural planes which lie substantially at 48° with respect to the optical axis of speed 20 of propagation of sound is 7700 meters. These widely varying constants are probably due to the fact that the material lying in these different planes have wide differences in the moduli of elasticity. The structure of 25 the crystal shows that the aforesaid planes lying at angles of approximately 70° and approximately 48° with respect to the optical axis have a crystalline structure which is unusually regular in its formation.

30 In accordance with the principles of this invention, therefore, a longitudinally vibrating crystal plate or rod, which has its longitudinal axis lying in either of the aforementioned planes, exhibits particularly perfect 35 and clear conditions of oscillations, whether used as a transmitter, or as a controlling element, or as a receiver. Also, crystal plates or rods cut with their longitudinal axis lying in planes at angles to the optical axis, as 40 pointed out above, are more readily excitable, and show greater responsiveness, and also display most efficiently the phenomenon common to piezo electric crystals at their natural periods.

45 The method which I employ in preparing crystals in accordance with this invention will be more readily understood from the following description taken in connection with the accompanying drawing in which:

50 Fig. 1 is a diagrammatic view showing the

orientation of the longitudinal axis of crystals, with respect to the optical axis, cut in accordance with this invention; and

Figs. 2 and 3 are perspective views of native quartz crystals having a top section which is cut along each of the above mentioned preferential planes.

Referring in detail to Fig. 1, OA indicates the optical axis of a native quartz crystal. PB indicates a plane at right angles to the plane of the paper and which is at an angle of 40° to 50° with respect to the optical axis OA of the native crystal. A quartz crystal oscillator plate or rod having its longitudinal axis lying in the plane PB and with its faces A'' and B'' at right angles and parallel respectively to the plane PB as shown in Fig. 1, will have the desirable features of a crystal as explained above. It will be understood that the point along the optical axis at which the plane PB is cut is practically immaterial, for the reason that most crystals have the preferential planes of structure described above throughout their length, and that a section cut at any point along the optical axis, at the angle indicated, will exhibit the desirable effects described.

In the same way I have found that a plane QR lying at an angle of 60° to 75° with respect to the optical axis will also be a preferential plane and a crystal having the dimensions a' b' as shown in Fig. 1 will also give improved results in operation either as a crystal oscillator or as a controlling element for a transmitter or receiver.

The plates a'' b'' and a' b' as shown, of course, are at the same time at right angles to one of the three electrical axes.

The crystal shown in dotted lines of Fig. 1 and having the dimensions a b show the prior art method of cutting the crystal and by comparison with the crystals a' b' and a'' b'' show the essential features of my improved method.

While I have disclosed the preferential planes as lying at angles of 40° to 50° and 60° to 70° with respect to the optical axis it is to be understood that in some crystals these planes might vary somewhat from these particular angles and that this disclosure is

therefore intended merely to indicate the order of magnitude of these angles and that in some cases it may be found that the preferential plane lies at an angle slightly displaced from the aforesaid angles.

Having thus described my invention, I claim:

1. A piezo-electric crystal element cut from a crystalline body at right angles to one of the electrical axes of said body, said body having an optical axis, said element having an axis of symmetry and strata of crystalline material lying in planes parallel to said axis of symmetry and disposed at an angle of  $60^{\circ}$  to  $75^{\circ}$  inclusive with respect to the said optical axis.
2. A piezo-electric crystal element cut from a crystalline body in a direction at right angles to one of the electrical axes of said body, said crystal having a longitudinal axis and an optical axis and being adapted to be stimulated electrically to produce longitudinal vibrations, said longitudinal axis lying at an angle of  $60^{\circ}$  to  $75^{\circ}$  with respect to said optical axis.
3. A piezo-electric crystal element cut from a crystalline body in a direction at right angles to one of the electrical axes of said body, said element being adapted to be stimulated electrically to vibrate mechanically, the longitudinal axis of said element lying in a plane of  $60^{\circ}$  to  $75^{\circ}$  with respect to the optical axis, said element being more readily excitable electrically and being more responsive to electrical stimulation than piezo-electric crystal elements of the same material and having their longitudinal axes at right angles to the optical axes.
4. A piezo-electrical crystal element cut from a crystalline body at right angles to one of the electrical axes of said body, said crystal having a longitudinal axis and an optical axis and being adapted to be stimulated electrically to produce longitudinal vibrations, said longitudinal axis lying at an angle of substantially  $67\frac{1}{2}^{\circ}$  with respect to said optical axis.
5. A parallelopiped piezo-electric element cut from a crystalline body having an optical axis and electrical axes in such manner that two faces of said element are at right angles to one of the electrical axes of said body, said element having an axis of symmetry and strata of crystalline material lying in planes parallel to said axis of symmetry, said axis of symmetry lying in a plane substantially  $67\frac{1}{2}^{\circ}$  with respect to the optical axis of said crystalline body.

ALEXANDER MEISSNER.